# EUROPEAN PATENT SPECIFICATION

(11) **EP 0 681 053 B1**
(45) Date of publication and mention of the grant of the patent: **07.11.2001**
(21) Application number: 94303133.6
(22) Date of filing: 29.04.1994
(51) Int. Cl.: D06M 14/10, D06M 14/04

(54) **Carboxyl group-modified cellulose or acryl fiber and process of producing same**
Carboxygruppenmodifizierte Cellulose- oder Acrylfasern und Verfahren zur Herstellung derselben
Fibres acryliques ou cellulosiques modifiées par des groupements carboxyl et procédé pour leur fabrication

(43) Date of publication of application: 08.11.1995
(73) Proprietor: NIPPON SANMO SENSYOKU CO.,LTD., Kyoto-shi, Kyoto (JP)
(72) Inventor: Gomibuchi, Reizo, Uji-shi, Kyoto-fu (JP)
(74) Representative: Allam, Peter Clerk

(56) References cited:
- EP-A- 0 189 163
- EP-A- 0 262 405
- FR-A- 2 384 867
- FR-A- 2 387 250
- US-A- 4 743 267
- TEXTILE RESEARCH JOURNAL., vol.59, no.9, September 1989, US pages 525 - 529, XP51475 J.DAS, A.K. MOHANTY AND B.C. SINGH 'Fenton's Reagent Initiated Graft Copolymerization of Methyl Methacrylate onto Jute Fibers'
- DATABASE WPI Week 9431, Derwent Publications Ltd., London, GB; AN 94-253428 & JP-A-6 184 941 (NIPPON SANMO SENSHOKU KK) 5 July 1994

## Description

This invention relates generally to a fiber modified with carboxyl groups and, more specifically, to an acrylonitrile fiber to which methacrylic acid or a hydroxyalkyl methacrylate is graft-copolymerized. The present invention is also directed to a process for producing such a modified fiber.

An acrylonitrile fiber has properties similar to wool but has a defect that its moisture or damp absorbing power is poor. No effective method is however known to impart hydrophilicity to the acrylonitrile fiber.

A method is known in which a vinyl monomer having an acidic group is graft-copolymerized to a polyester or polyamide fiber using an organic peroxide such as benzoyl peroxide.

EP-A-0262405 discloses a process for preparing a water absorptive composite material in which an aqueous solution of a polymerizable monomer comprising acrylic acid (at least partly in the form of alkali metal or ammonium salts) is applied to a prefabricated fibrous substrate, polymerized in situ and then crosslinked by the addition of a crosslinking agent to the composite. The polymerizable monomer may also contain up to 20 mol % of optional comonomers and methacrylic acid, 2-hydroxyethyl methacrylate and 2-hydroxypropyl methacrylate are mentioned in that connection. The substrate material is preferably a cellulose or polyester fiber but may also be polyacrylonitrile.

Textile Research Journal, 1989, (59), pages 525-529 reports a study of the graft copolymerization of methyl methacrylate onto chemically modified jute fibers using Fenton's reagent (Fe⁺⁺/H₂O₂).

In accordance with the present invention there is provided a modified fiber comprising an acrylonitrile-series substrate fiber and a graft comonomer graft-copolymerized to said substrate fiber in an amount of 3-60% by weight based on the weight of said substrate fiber, said graft comonomer being at least one member selected from methacrylic acid and hydroxyalkyl methacrylate.

In another aspect, the present invention provides a process for the production of a modified fiber, comprising graft-copolymerizing a graft comonomer to an acrylonitrile-series substrate fiber in an aqueous medium containing hydrogen peroxide and a source of ferrous ion, said graft comonomer being at least one member selected from methacrylic acid and hydroxyalkyl methacrylates.

The present invention will now be described in detail below.

The acrylonitrile fiber used in the present invention, may be in any desired form such as a yarn, a cotton, a woven or non-woven fabric, a filament or a tow. If desired, the substrate fiber may be used in combination with another fiber. The term "acrylonitrile-series fiber" used in the present specification and claims is intended to refer to a fiber formed of a homopolymer acrylonitrile or a copolymer of acrylonitrile with a vinyl comonomer. Examples of the vinyl comonomers include methyl acrylate, vinyl acetate, acrylic acid, methacrylic acid, vinyl chloride, vinylidene chloride, methylvinylpyridine, styrenesulfonic acid and mixtures thereof. The copolymer of acrylonitrile with the vinyl comonomer generally has a content of the acrylonitrile of at least 20% by weight, preferably 35-90% by weight.

To the substrate fiber is graft-copolymerized and linked a graft comonomer in an amount of 3-60% by weight based on the weight of the substrate fiber. The graft comonomer is selected from acrylic acid and hydroxyalkyl methacrylate such as 2-hydroxyethyl methacrylate and 2-hydroxypropyl methacrylate. The graft comonomer is preferably copolymerized in an amount of 5-40% by weight.

The modified fiber according to the present invention may be prepared by graft-copolymerizing the graft comonomer to the substrate fiber in an aqueous medium containing hydrogen peroxide and a source of ferrous ion.

The ferrous ions source is preferably a ferrous salt such as ferrous sulfate, ferrous chloride, ammonium ferrous sulfate or ferrous nitrate. The ferrous in salt is preferably present in the aqueous medium in an amount providing a ferrous ion concentration of 0.5 to 5 mmol/liter, more preferably 0.7 to 1.6 mmol/liter.

The concentration of the hydrogen peroxide in the aqueous medium is preferably 0.01 to 0.1 mol/liter, more preferably 0.01 to 0.06 mol/liter. The hydrogen peroxide and the ferrous ion source together serve to accelerate the graft copolymerization.

The aqueous medium may contain an acid in an amount of 2 to 4 mmol/liter, preferably 2.5 to 3.5 mmol/liter, if desired. The acid serves to enhance the grafting rate of the graft comonomer. Examples of suitable acids include sulfuric acid, hydrochloric acid, phosphoric acid and formic acid. Further, the aqueous medium may further contain a sequestering agent such as EDTA, NTA or a phosphoric acid-type or sulfonic acid-type agent.

The graft comonomer is generally used in an amount of 5-100 parts by weight, preferably 10-60 parts by weight, per 100 parts by weight of the substrate fiber and wherein the weight ratio of said aqueous medium to said substrate fiber is generally 5:1 to 50:1, preferably 5:1 to 15:1.

The graft copolymerization is generally performed at a temperature and for a period of time so that the graft monomer is grafted to the substrate fiber in an amount of 3-60% by weight based on the weight of the substrate fiber. Preferably, the graft degree (weight percentage of the grafted comonomer based on the weight of the substrate fiber) is 5-40% by weight when a methacrylonitrile-series fiber is used as the substrate fiber. The graft copolymerization is generally performed at a temperature of 40°-110°C for 30-240 minutes, preferably at 70°-110°C for 30-180 minutes, more preferably 90°-100° for 60-90 minutes.

If desired, the carboxy groups (-COOH) introduced into the substrate fiber by graft copolymerization of the graft comonomer may be converted into -COOM (M represents a cation) by reaction with a salt-forming cation. The cation may be, for example, sodium ion, calcium ion, ferrous ion, cupric ion, zinc ion, manganese ion, silver ion, quaternary ammonium ion or quaternary organic amine ion.

The process according to the present invention uses a ferrous salt in a very small amount. Therefore, the modified fibers are not discolored and no specific step for the removal of the ferrous salt is required. Further, the reaction conditions for the modification treatment may be easily controlled so that the graft copolymerization can be homogeneously performed.

The modified fibers of the present invention have improved hydrophilicity and serve to function as a good adsorbent not only for basic, bad odor substances such as ammonia and amines, but also for metal ions.

The following examples will further illustrate the present invention. Percentages are by weight.

### Example 1

Into an aqueous solution (150 ml) containing 0.3 % of hydrogen peroxide, 0.02 % of ferrous sulfate, 1.5 % of methacrylic acid, 0.03 % a sequestering agent (Chelest NTB) and 0.06 % of sulfuric acid (50°Be), 10 g of acrylic fibers (Cashimiron 3Dx76V GK manufactured by Asahi Kasei Kogyo Co., Ltd.) were immersed. The mixture was gradually heated from room temperature to 100°C and maintained at that temperature for 1 hour. The treated fibers were washed well with water and dried to obtain modified acrylic fibers having a graft degree of 10.6 %.

### Example 2

Into an aqueous solution (100 ml) containing 0.5 % of hydrogen peroxide, 0.02 % of ferrous sulfate, 2.5 % of methacrylic acid, 0.05 % a sequestering agent (Chelest NTB) and 0.1 % of sulfuric acid (50°Be), 10 g of acrylic fibers (Kanebo Acryl WQ-1 1.8Dx76 mm, manufactured by Kanebo Co., Ltd.) were immersed. The mixture was gradually heated from room temperature to 100°C and maintained at that temperature for 1 hour. The treated fibers were washed well with water and dried to obtain modified acrylic fibers having a graft degree of 10.1 %.

### Example 3

Into an aqueous solution (150 ml) containing 0.5 % of hydrogen peroxide, 0.02 % of ferrous sulfate, 3 % of methacrylic acid, 0.05 % a sequestering agent (Chelest NTB) and 0.05 % of sulfuric acid (50°Be), 10 g of acrylic fibers (Toraylon 5x18 mm, manufactured by Toray Co., Ltd.) were immersed. The mixture was gradually heated from room temperature to 100°C and maintained at that temperature for 1 hour. The treated fibers were washed well with water and dried to obtain modified acrylic fibers having a graft degree of 9.6 %.

### Example 4

Example 3 was repeated in the same manner as described except that modacrylic fibers (Kanebo Acryl VE1 manufactured by Kanebo Co., Ltd.) was substituted for Toraylon. The modified acrylic fibers thus obtained had a graft degree of 8.1 %.

### Example 5

Example 1 was repeated in the same manner as described except that 2-hydroxyethyl methacrylate was substituted for methacrylic acid. The modified acrylic fibers thus obtained had a graft degree of 9.3 %.

### Example 6

Into an aqueous solution (100 ml) containing 0.5 % of hydrogen peroxide, 0.02 % of ferrous sulfate, 1.5 % of methacrylic acid, 1.5 % of 2-hydroxyethyl methacrylate, 0.05 % a sequestering agent (Chelest NTB) and 0.1 % of sulfuric acid (50°Be), 10 g of acrylic yarn (Silpalon 100d/-48f, manufactured by Mitsubishi Rayon Co., Ltd.) were immersed. The mixture was gradually heated from room temperature to 100°C and maintained at that temperature for 1 hour. The treated fibers were washed well with water and dried to obtain modified acrylic yarn weighing 114 % of the raw mterial yarn. The analysis of the carboxylic group revealed that the modified yarn had a grafted methacrylic acid monomber content of 6.4 %.

## Claims

1. A modified fiber, comprising an acrylonitrile-series substrate fiber and a graft comonomer graft-copolymerized to said substrate fiber in an amount of 3-60% by weight based on the weight of said substrate fiber, said graft comonomer being at least one member selected from methacrylic acid and hydroxyalkyl methacrylate.

2. A modified fiber as claimed in Claim 1, wherein said acrylonitrile-series fiber is a fiber formed of a homopolymer of acrylonitrile or a copolymer of acrylonitrile with a vinyl comonomer.

3. A modified fiber as claimed in Claim 2, wherein said vinyl comonomer is selected from methyl acrylate, vinyl acetate, acrylic acid, methacrylic acid, vinyl chloride, vinylidene chloride, methylvinylpyridine and styrenesulfonic acid.

4. A modified fiber as claimed in Claim 2 or Claim 3, wherein said copolymer has an acrylonitrile content of at least 20% by weight.

5. A modified fiber as claimed in any preceding claim, wherein said hydroxyalkyl methacrylate is 2-hydroxyethyl methacrylate or 2-hydroxypropyl methacrylate.

6. A process for the production of a modified fiber as defined in Claim 1, comprising graft-copolymerizing a graft comonomer to an acrylonitrile-series substrate fiber in an aqueous medium containing hydrogen peroxide and a source of ferrous ion, said graft comonomer being at least one member selected from methacrylic acid and hydroxyalkyl methacrylates.

7. A process as claimed in Claim 6, wherein said source of ferrous ion is a ferrous salt.

8. A process as claimed in Claim 7, wherein said ferrous salt is selected from ferrous sulfate, ferrous chloride, ammonium ferrous sulfate and ferrous nitrate.

9. A process as claimed in Claim 7 or Claim 8, wherein said ferrous salt and said hydrogen peroxide are present in said aqueous medium in amounts of 0.5 to 5 mmol/liter and 0.01 to 0.1 mol/liter, respectively.

10. A process as claimed in any one of Claims 6-9, wherein said graft comonomer is used in an amount of 5-100 parts by weight per 100 parts by weight of said substrate fiber, and wherein the weight ratio of said aqueous medium to said substrate fiber is from 5:1 to 50:1.

11. A process as claimed in any one of Claims 6-10, wherein said graft copolymerization is performed at a temperature of 40°-110°C for a period of time so that said graft monomer is grafted to said substrate fiber in an amount of 3-60% by weight based on the weight of said substrate fiber.

## Patentansprüche

1. Modifizierte Faser, umfassend eine Trägerfaser der Acrylnitrilreihe und ein Pfropfcomonomer, das in einer Menge von 3-60 Gew.-% auf der Basis des Gewichts der genannten Trägerfaser auf die genannte Trägerfaser aufcopolymerisiert wird, wobei das genannte Pfropfcomonomer wenigstens ein Element ausgewählt aus Methacrylsäure und Hydroxyalkylmethacrylat ist.

2. Modifizierte Faser nach Anspruch 1, wobei die genannte Faser der Acrylnitrilserie eine Faser ist, die aus einem Acrylnitril-Homopolymer oder einem Acrylnitril-Copolymer mit einem Vinylcomonomer gebildet ist.

3. Modifizierte Faser nach Anspruch 2, wobei das genannte Vinylcomonomer aus Methylacrylat, Vinylacetat, Acrylsäure, Methacrylsäure, Vinylchlorid, Vinylidenchlorid, Methylvinylpyridin und Styren-Sulfonsäure ausgewählt ist.

4. Modifizierte Faser nach Anspruch 2 oder Anspruch 3, wobei das genannte Copolymer einen Acrylnitrilgehalt von wenigstens 20 Gew.-% hat.

5. Modifizierte Faser nach einem der vorherigen Ansprüche, wobei das genannte Hydroxyalkylmethacrylat 2-hydroxyethylmethacrylat oder 2-hydroxypropylmethacrylat ist.

6. Verfahren zur Herstellung einer modifizierten Faser nach Anspruch 1, umfassend das Aufcopolymerisieren eines Pfropfcomonomers auf eine Trägerfaser der Acrylnitrilserie in einem wässrigen Medium, das Wasserstoffperoxid und eine Eisen(II)-Ionenquelle enthält, wobei das genannte Pfropfcomonomer wenigstens ein Element ausgewählt aus Methacrylsäure und Hydroxyalkylmethacrylaten ist.

7. Verfahren nach Anspruch 6, wobei die Eisen(II)-Ionenquelle ein Eisen(II)-Salz ist.

8. Verfahren nach Anspruch 7, wobei das genannte Eisen(II)-Salz ausgewählt ist aus Eisen(II)-Sulfat, Eisen(II)-Chlorid, Ammonium-Eisen(II)-Sulfat und Eisen(II)-Nitrat.

9. Verfahren nach Anspruch 7 oder Anspruch 8, wobei das genannte Eisen(II)-Salz und das genannte Wasserstoffperoxid in Mengen von jeweils 0,5 bis 5 mmol/Liter und 0,01 bis 0,1 mol/Liter in dem genannten wässrigen Medium vorliegen.

10. Verfahren nach einem der Ansprüche 6-9, wobei das genannte Pfropfcomonomer in einer Menge von 5-100 Gewichtsteilen pro 100 Gewichtsteile der genannten Trägerfaser eingesetzt wird und wobei das Gewichtsverhältnis des genannten wässrigen Mediums zu der genannten Trägerfaser zwischen 5:1 und 50:1 liegt.

11. Verfahren nach einem der Ansprüche 6-10, wobei die genannte Aufcopolymerisation bei einer Temperatur von 40°-110°C für eine Zeitdauer durchgeführt wird, die ausreicht, damit das genannte Pfropfmonomer in einer Menge von 3-60 Gew.-% auf der Basis des Gewichts der genannten Trägerfaser auf diese aufgepfropft wird.

## Revendications

1. Fibre modifiée, comprenant une fibre de substrat de la série de l'acrylonitrile et un comonomère greffé copolymérisé par greffage à ladite fibre de substrat en une quantité de 3 à 60% en poids sur la base du poids de ladite fibre de substrat, ledit comonomère greffé étant au moins un membre sélectionné parmi l'acide méthacrylique et le méthacrylate d'hydroxyalkyle.

2. Fibre modifiée selon la revendication 1, dans laquelle ladite fibre de la série de l'acrylonitrile est une fibre formée par un homopolymère d'acrylonitrile ou par un copolymère d'acrylonitrile avec un comonomère vinylique.

3. Fibre modifiée selon la revendication 2, dans laquelle ledit comonomère vinylique est sélectionné parmi l'acrylate de méthyle, l'acétate de vinyle, l'acide acrylique, l'acide méthacrylique, le chlorure de vinyle, le chlorure de vinylidène, la méthylvinylpyridine et l'acide styrènesulfonique.

4. Fibre modifiée selon la revendication 2 ou la revendication 3, dans laquelle ledit copolymère a une teneur en acrylonitrile d'au moins 20% en poids.

5. Fibre modifiée selon l'une quelconque des revendications précédentes, dans laquelle ledit méthacrylate d'hydroxyalkyle est le méthacrylate de 2-hydroxyéthyle ou le méthacrylate de 2-hydroxypropyle.

6. Procédé de production d'une fibre modifiée telle que définie dans la revendication 1, comprenant la copolymérisation par greffage d'un comonomère de greffage à une fibre de substrat de la série de l'acrylonitrile dans un milieu aqueux contenant du peroxyde d'hydrogène et une source d'ions ferreux, ledit comonomère de greffage étant au moins un membre sélectionné parmi l'acide méthacrylique et les méthacrylates d'hydroxyalkyle.

7. Procédé selon la revendication 6, dans lequel ladite source d'ions ferreux est un sel ferreux.

8. Procédé selon la revendication 7, dans lequel ledit sel ferreux est sélectionné parmi le sulfate ferreux, le chlorure ferreux, le sulfate d'ammonium ferreux et le nitrate ferreux.

9. Procédé selon la revendication 7 ou la revendication 8, dans lequel ledit sel ferreux et ledit peroxyde d'hydrogène sont présents dans ledit milieu aqueux en des quantités de 0,5 à 5 mmol/litre et de 0,01 à 0,1 mol/litre, respectivement.

10. Procédé selon l'une quelconque des revendications 6 à 9, dans lequel ledit comonomère de greffage est utilisé en une quantité de 5 à 100 parties en poids par 100 parties en poids de ladite fibre de substrat, et dans lequel le rapport pondéral dudit milieu aqueux à ladite fibre de substrat est de 5:1 à 50:1.

11. Procédé selon l'une quelconque des revendications 6 à 10, dans lequel ladite copolymérisation de greffage est réalisée à une température de 40° à 110°C pour une période de temps telle que ledit monomère de greffage est greffé sur ladite fibre de substrat en une quantité de 3 à 60% en poids sur la base du poids de ladite fibre de substrat.
